

1

3,567,454

### LIGHT-SENSITIVE MATERIALS

Jozef Frans Willems, Wilrijk, Robrecht Julius Thiers, Brasschaat, and Adam Marcel Schouwenaars, Edegem, Belgium, assignors to Gevaert-Agfa N.V., Mortsel, Belgium  
No Drawing. Filed Nov. 21, 1967, Ser. No. 684,622  
Claims priority, application Great Britain, Dec. 12, 1966, 55,445/66

Int. Cl. G03c 1/34

U.S. Cl. 96—109

7 Claims

### ABSTRACT OF THE DISCLOSURE

Photographic materials comprising a support and at least one layer of light-sensitive silver halide emulsion containing a water-soluble mercury(II) compound having one of the following formulae:



wherein:

$X_1$  is a bivalent organic radical,  
 $X_2$  stands for an aliphatic or aromatic bivalent group,  
 $M$  represents hydrogen, alkali metal, alkaline earth metal, ammonium, guanidine or an organic amine, and  
 $Y$  stands for an aliphatic, alicyclic, aromatic or heterocyclic radical, said radicals including the substituted derivatives thereof

are described. The photographic material has improved stability and fogging characteristics.

This invention relates to improved light-sensitive silver halide emulsions.

Light-sensitive silver halide emulsions are in general characterised by their sensitivity, gradation and fog.

As is well-known, sensitivity, gradation and fog are determined by the way in which the silver halide emulsion is prepared and by the use of special chemical ingredients effecting a desired improvement or result. Addenda to the emulsion, which are of particular importance for the stability of the light-sensitive characteristics of a silver halide emulsion are the so-called "stabilizers."

Stabilizers or antifogging agents protect the light-sensitive silver halide emulsions against spontaneous formation and growth of fog known as chemical fog during prolonged storage or storage at high temperatures and humidities or during development to maximum contrast and speed. Indeed, the fog increases with the degree and temperature of development, and, in constant development circumstances, with the time the light-sensitive emulsion is stored and with the temperature and the relative humidity of the atmosphere wherein the emulsion is stored. It is evident that a light-sensitive emulsion should be obtained which is as stable as possible at high temperature and high relative humidity for instance in view of its use in tropical countries.

It is known to protect light-sensitive silver halide emulsions against the growth of chemical fog during storage by addition of stabilizers of the triazolopyrimidine type (azaindolizines). Heterocyclic thioxo and mercapto compounds too have been proposed for this purpose but show the disadvantage of impairing the sensitivity and gradation. The same disadvantageous influence on the sensitivity occurs with the known mercury compounds such as simple anorganic mercury salts, addition com-

2

plexes of mercury with amines, organic mercury salts and heterocyclic mercury compounds. Indeed, these compounds, when used in the concentration necessary for obtaining a sufficient antifogging action, have a considerable desensitizing effect.

It is also known that emulsions stabilised with compounds of the triazolopyrimidine type still show a tendency to fog formation in extreme storage circumstances i.e. at very high temperatures and humidities and in extreme development circumstances e.g. rapid processing at elevated temperatures. The addition to these emulsions of the above known mercury compounds reduces the fogging tendency but, as mentioned above, at the cost of a reduction of the sensitivity.

It has now been found that mercury(II) compounds corresponding to one of the following general Formulae I and II



20 wherein:

$X_1$  represents a bivalent organic radical e.g. an aliphatic, aromatic or heterocyclic bivalent radical such as alkylene including substituted alkylene, arylene including substituted aralkylene and a bivalent radical comprising a heterocyclic nucleus including a substituted heterocyclic nucleus,

$X_2$  stands for an aliphatic or aromatic bivalent group such as alkylene including substituted alkylene, arylene including substituted arylene, and aralkylene including substituted aralkylene,

$M$  represents hydrogen, an alkali metal or alkaline earth metal, ammonium, guanidine, an organic amine, etc., and

35  $Y$  stands for an organic aliphatic, alicyclic, aromatic or heterocyclic radical said radicals including the substituted alkyl, aryl including substituted aryl and a heterocyclic nucleus including a substituted heterocyclic nucleus,

40 are particularly good stabilizers and antifoggants for photographic light-sensitive silver halide emulsions without causing an appreciable desensitization of the light-sensitive silver halide emulsion material.

45 Moreover, it has been found that these mercury(II) compounds are very suitable for use in combination with stabilizers of the triazolopyrimidine type, particularly in extreme storage and development circumstances in order to reduce the fogging tendency of the light-sensitive emulsion without giving rise to an appreciable desensitization thereof.

50 The high-water-solubility, obtained by the presence of the sulphonate acid group in the mercury(II) compounds of the above general formula guarantees a homogeneous distribution of the stabilizer in the emulsion.

55 The following is a non-limitative list of particularly suitable mercury(II) compounds for use as stabilizers for photographic light-sensitive silver halide emulsions according to the present invention:





The watersoluble mercury(II) mercaptides of use according to the present invention can be prepared by allowing to react a mercury(II) salt such as mercury(II) acetate or mercury(II) chloride with the corresponding mercapto compound. The said mercury(II) mercaptides can also be obtained in a very pure form by reaction of mercury(II) oxide with the corresponding mercapto compound.

The mercury(II) compounds corresponding to the above general Formula II can be prepared by allowing to react the corresponding organo-mercury salts such as the chlorides, bromides or acetates or the corresponding organomercury hydroxides with the sulphonated mercaptans.

The following preparations illustrate more particularly how the mercury(II) compounds are prepared.

#### PREPARATION 1.—COMPOUND 1

(a) To a solution of 10.75 g. (0.05 mole) of the guanidine salt of 3-mercaptopropane sulphonlic acid in 55 ccs. of water a solution of 7.95 g. (0.025 mole) of mercury(II) acetate in 35 ccs. of water was added. The water was distilled off under reduced pressure and the mercury(II) mercaptide formed was recrystallized from methanol.

(b) To a solution of 43 g. (0.2 mole) of the guanidine salt of 3-mercaptopropane sulphonlic acid in 500 ccs. of water, 21.6 g. (0.1 mole) of yellow mercury(II) oxide

#### 4

were added with vigorous stirring. After evaporation of the water the residue was washed with acetone.

#### PREPARATION 2—COMPOUND 3

5 To a solution of 13.15 g. (0.05 mole) of the guanidine salt of o-sulpho-benzyl mercaptan in 300 ccs. of water a solution of 7.95 g. (0.025 mole) of mercury(II) acetate in 50 ccs. of water was added. A white precipitate formed, which was filtered by suction and washed with alcohol.

#### PREPARATION 3.—COMPOUND 4

15 To a solution of 12.8 g. (0.05 mole) of the guanidine salt of 2-mercaptop-4-methyl-4-sulpho-pentane in 400 ccs. of water a solution of 7.95 g. (0.025 mole) of mercury(II) acetate in 50 ccs. of water was added. After evaporation of the water the residue was digested with methanol and dried.

#### PREPARATION 4.—COMPOUND 5

20 To a solution of 7.7 g. (0.03 mole) of 5-(m-sulphophenyl)-triazoline-3-thione in 100 ccs. of water a solution of 4.78 g. (0.015 mole) of mercury(II) acetate in 25 ccs. of water was added. The precipitate formed was 25 filtered by suction and washed with water and ethanol. The mercury(II) mercaptide formed is soluble in diluted sodium hydroxide.

#### PREPARATION 5.—COMPOUND 7

30 (a) 79 g. of mercury(II) acetate, 15.5 g. of allyl alcohol and 150 ccs. of methanol were refluxed for 5 min. The excess of methanol and the acetic acid formed were distilled off under reduced pressure. The product obtained (32 g.) had an oxygen content of 18.76% 35 (calculated: 18.4%).

(b) 3.48 g. of the product obtained in (a) were treated with an aqueous solution of 2.15 g. of the guanidine salt of 3-mercaptopropane sulphonlic acid. The water was distilled off under reduced pressure and the 40 residue purified with ethanol.

#### PREPARATION 6.—COMPOUND 8

A solution of 10 g. of allylurea in 120 ccs. of methanol, 31.9 g. of mercury(II) acetate and 6 ccs. of acetic acid were refluxed for 6 hours. The excess of methanol and the acetic acid formed were distilled off under reduced pressure.

To the residue an aqueous solution of 21.5 g. of the guanidine salt of 3-mercaptopropane sulphonlic acid was 50 added with vigorous stirring. The mercury(II) compound formed was purified with ethanol.

#### PREPARATION 7.—COMPOUND 12

(a) To a solution of 13.5 g. of mercury(II) chloride 55 in 200 ccs. of water a solution of 6 g. of sodium hydroxide in 25 ccs. of water was added. The precipitate formed was filtered off by suction and washed with water until no chloride ions could be indicated anymore.

The product was suspended in 50 ccs. of water and 60 then an aqueous solution of 22 g. of salicylic acid was added with stirring. After some hours the suspension formed was concentrated by evaporation and the residue digested with ethanol.

(b) 4.3 g. of the compound obtained according to (a) 65 were treated with an aqueous solution of 1.8 g. of the sodium salt of 3-mercaptopropane sulphonlic acid. After having concentrated the solution by evaporation the residue was purified with ethanol.

As compared with the known mercury compounds used 70 as stabilizers the mercury(II) compounds according to the present invention when used in the appropriate concentration do not cause or only to a slight extent a decrease in sensitivity.

The antifoggants according to the present invention 75 are particularly suitable for use in combination with com-

pounds which sensitize the emulsion by development acceleration for example compounds of the polyoxyalkylene type such as alkylene oxide condensation products as described among others in United States Pat. 2,531,832 and 2,533,990, in United Kingdom Pat. 920,637, 940,051, 945,340 and 991,608 and in Belgian Pat. 648,710 and onium derivatives of amino-N-oxides as described in U.S. patent application Ser. No. 573,801, filed Aug. 22, 1966, and now pending.

The stabilizers according to the inventions can also be used in combination with other known stabilizers for instance with heterocyclic nitrogen containing thioxo compounds such as benzothiazoline-2-thione and 1-phenyl-2-tetrazoline-5-thione and, as said above, preferably with compounds of the hydroxytriazolopyrimidine type (azaindolizines).

The stabilizers according to the present invention may be incorporated into any type of light-sensitive material comprising a silver halide emulsion layer e.g. a spectrally sensitized or non-sensitized emulsion layer, X-ray emulsion layer, and an emulsion layer sensitive to infra-red radiation. They may be incorporated into high-speed negative materials as well as into rather low speed positive materials. Various silver salts may be used as light-sensitive salt e.g. silver bromide, silver iodide, silver chloride, or mixed silver halides e.g. silver chloro-bromoide or silver bromo-iodide.

The silver halides are dispersed in the common hydrophilic colloids such as gelatin, casein, zein, polyvinyl alcohol, carboxymethylcellulose, alginic acid, etc., gelatin being however favoured.

The stabilizing agents are generally incorporated into the silver halide emulsion layer of the light-sensitive material; they may be added to the emulsion during no matter what step of emulsion preparation; however, they are preferably added to the photographic emulsion after the chemical ripening and just before coating of the emulsion. The addenda according to the present invention are incorporated into the photographic emulsions according to the methods well known in emulsion preparation. For instance they can be added to the emulsion in the form of a solution or of a dispersion according to the methods applied for incorporating colour couplers in the emulsion. Instead of incorporating the compounds of the invention into the emulsion layer they can also be incorporated into a water-permeable layer e.g. a gelatin covering layer or intermediate layer.

The amount of mercury(II) compound employed in the light-sensitive silver halide material depends on the particular type of emulsion and the desired effect and can vary within very wide limits. The optimum amount of mercury(II) compound to be added can be determined for each particular emulsion in a very simple way by application of the usual tests. Usually said compounds are employed in a ratio of about 0.1 mg. to about 30 mg. per mole of silver halide.

The light-sensitive emulsions may be chemically as well as optically sensitized. They may be chemically sensitized by effecting the ripening in the presence of small amounts of sulphur containing compounds such as allylthiocyanate, allyl thiourea, sodium thiosulphate, etc. The emulsions may also be sensitized by means of reductors for instance tin compounds as described in our French patent specification 1,146,955 and in our Belgian patent specification 568,687, imino-aminomethane sulphonic acid compounds as described in our British patent specification 789,823 and small amounts of noble metal compounds such as of gold, platinum, palladium, iridium, ruthenium and rhodium.

Other addenda such as hardening agents, wetting agents, plasticizers, colour couplers, developing agents and optical sensitizers can be incorporated into the emulsion in the usual way.

The following examples illustrate the present invention.

A high sensitive gelatino silver bromoiodide emulsion ( $\pm 4.5$  mole percent of iodide) is divided into six aliquot portions A, B, C, D, E and F.

5 To emulsion portion B is added per mole of silver halide  $1.2 \times 10^{-2}$  millimole (3 mg.) of mercury (II) cyanide, to emulsion portion C  $0.6 \times 10^{-2}$  millimole (3.8 mg.) of compound 1, to emulsion portion D  $1.2 \times 10^{-2}$  millimole (7.5 mg.) of compound 1, to emulsion portion E  $2.0 \times 10^{-2}$  millimole (10 mg.) of compound 7 and to emulsion portion F  $1.2 \times 10^{-2}$  millimole (6.6 mg.) of compound 8. The six emulsions are then coated on a subbed cellulose triacetate support and dried whereupon the six materials thus obtained are stored for 5 days in an atmosphere of  $57^\circ \text{C}$ . and 34% of relatively humidity.

10 The stored materials as well as six identical freshly prepared materials are exposed and developed for 5 minutes at  $20^\circ \text{C}$ . in a developing bath with the following composition:

20 Water—800 ccs.  
p-Monomethylaminophenol sulphate—1.5 g.  
Sodium sulphite (anhydrous)—50 g.  
Hydroquinone—6 g.  
25 Sodium carbonate (anhydrous)—32 g.  
Potassium bromide—2 g.  
Water up to—1000 ccs.

30 After the treatment in a stop bath, rinsing and fixing of the materials the following sensitometric results are obtained.

TABLE

| Material | Freshly prepared materials |                      |                | Stored materials |                      |
|----------|----------------------------|----------------------|----------------|------------------|----------------------|
|          | Fog                        | Grada-tion (percent) | Relative speed | Fog              | Grada-tion (percent) |
| A        | 0.05                       | 1.42                 | 100            | 0.53             | 1.18                 |
| B        | 0.04                       | 1.36                 | 26             | 0.05             | 1.38                 |
| C        | 0.04                       | 1.45                 | 78             | 0.04             | 1.47                 |
| D        | 0.04                       | 1.47                 | 45             | 0.04             | 1.41                 |
| E        | 0.04                       | 1.57                 | 64             | 0.04             | 1.56                 |
| F        | 0.04                       | 1.61                 | 78             | 0.05             | 1.53                 |

35 The speed is given in relative values (i.e. in percent in respect of the absolute speed of an emulsion to which no mercury (II) compound was added. From this example it clearly appears that the mercury (II) compounds according to general formulae Ia and Ib have a markedly less desensitizing effect than the common organic mercury salts.

## Example 2

50 A gelatino silverbromoidide emulsion (0.35 mole percent of iodide) comprising per mole of silver halide 400 mg. of 5 - methyl - 7 - hydroxy-s-triazolo - [1,5-a] - pyrimidine and 5 mg. of 1-phenyl-2-tetrazoline - 5-thione as stabilizers, 200 mg. of development accelerator corresponding to the formula:



55 60 wherein  $x$  has a value of about 135 and 2 g. of saponin as coating aid, is divided into 4 aliquot portions.

To three of these emulsion portions is added an amount of compound 1 as listed in the table below.

65 The four emulsions are coated on both sides of a cellulose triacetate support, which has been provided on both sides with a subbing layer, in such a way that per sq. m. an amount of silver halide equivalent to 36 g. of silver nitrate (both sides taken together) is present.

The emulsion layers are then overcoated with a gelatin 70 antistress layer.

The four materials A, B, C and D obtained are then stored for 36 hours in an atmosphere of  $57^\circ \text{C}$ . and 34% of relative humidity.

75 Thereupon the said four materials as well as four identical freshly prepared materials are exposed to X-rays

with an X-ray radiation source of 80 kv. and developed for 8 min. at 20° C. in a common X-ray developer having the following composition:

Water—800 ccs.  
p-Monomethylaminophenol hemisulphate—4 g.  
Hydroquinone—10 g.  
Anhydrous sodium sulphite—65 g.  
Anhydrous sodium carbonate—45 g.  
Potassium bromide—5 g.  
Water up to—1000 ccs.

The results obtained are listed in the following table.

TABLE

| Material | Amount of stabilizer per mole of silver halide, mg. | Freshly prepared materials |                      | Fog produced in stored materials |
|----------|-----------------------------------------------------|----------------------------|----------------------|----------------------------------|
|          |                                                     | Fog                        | Relative sensitivity |                                  |
| A        | None                                                | 0.08                       | 100                  | 0.36                             |
| B        | 3                                                   | 0.08                       | 112                  | 0.24                             |
| C        | 6                                                   | 0.08                       | 112                  | 0.10                             |
| D        | 15                                                  | 0.05                       | 100                  | 0.04                             |

## Example 3

A gelatino silverbromiodide emulsion as described in Example 2 is divided into 4 aliquot portions.

To three of these emulsion portions is added an amount of mercury(II) compound as listed in the table below.

The four emulsions are then coated as described in Example 2 on a cellulose triacetate support and the resulting materials A, B, C and D are further treated as described in Example 2 with the difference, however, that the development now takes place at 26° C.

The results obtained are listed in the following table.

TABLE

| Material | Amount of mercury(II) mercaptide per mole of silver halide | Fog produced on development for 8 min. at 26° C. |                |
|----------|------------------------------------------------------------|--------------------------------------------------|----------------|
|          |                                                            | Fog                                              | Relative speed |
| A        | None                                                       | 0.44                                             |                |
| B        | 2.5 mg. of compound 1                                      | 0.30                                             |                |
| C        | 2.9 mg. of compound 3                                      | 0.30                                             |                |
| D        | 2.8 mg. of compound 4                                      | 0.28                                             |                |

## Example 4

A gelatino silverbromiodide emulsion as described in Example 2 is divided into 8 aliquot portions.

To seven of these emulsion portions is added an amount of mercury(II) compound as listed in the table below.

The eight emulsions are then further treated as described in Example 2 and the resulting materials are conditioned in a moist atmosphere of about 100% of relative humidity. Thereupon the materials are packed in aluminium, laminated paper and stored for 1 week at 57° C.

The following sensitometric results are obtained.

TABLE

| Material | Amount of mercury(II) mercaptide per mole of silver halide | Freshly prepared materials |                     |                |
|----------|------------------------------------------------------------|----------------------------|---------------------|----------------|
|          |                                                            | Fog                        | Gradation (percent) | Relative speed |
| A        | None                                                       | 0.11                       | 2.32                | 100            |
| B        | 2.5 mg. of compound 1                                      | 0.11                       | 2.10                | 99             |
| C        | 2.9 mg. of compound 3                                      | 0.11                       | 2.25                | 99             |
| D        | 2.8 mg. of compound 4                                      | 0.12                       | 2.21                | 100            |
| E        | 2.3 mg. of compound 7                                      | 0.12                       | 2.23                | 102            |
| F        | 2.3 mg. of compound 8                                      | 0.11                       | 2.20                | 99             |
| G        | 2.3 mg. of compound 10                                     | 0.11                       | 2.21                | 99             |
| H        | 2.3 mg. of compound 12                                     | 0.12                       | 2.24                | 102            |

We claim:

1. Photographic material comprising a support and at

least one light-sensitive silver halide emulsion layer comprising in said emulsion layer or in at least one water-permeable layer coated at the same side of the support as the said emulsion layer at least one water-soluble mercury(II) compound corresponding to one of the general Formulae I and II:



I

II

10 wherein:

$\text{X}_1$  is a bivalent organic radical,  
 $\text{X}_2$  stands for an aliphatic or aromatic bivalent group,  
 $\text{M}$  represents hydrogen, alkali metal, alkaline earth metal,  
15 ammonium, guanidine or an organic amine, and  
 $\text{Y}$  stands for an aliphatic, alicyclic, aromatic or heterocyclic radical, said radicals including the substituted derivatives thereof,

said mercury(II) compound being present in an amount  
20 sufficient to improve the stability or fogging characteristics of said material without appreciable desensitization thereof.

2. Photographic material according to claim 1, wherein  
25 in said mercury(II) compound corresponds to the formula:



wherein  $\text{X}_1$  stands for alkylene including substituted alkylene, arylene including substituted arylene, aralkylene including substituted aralkylene or a bivalent group comprising a heterocyclic nucleus including a substituted heterocyclic nucleus, and  $\text{M}$  represents hydrogen, alkali metal, alkaline earth metal, ammonium, guanidine or an organic amine.

3. Photographic material according to claim 1, wherein  
35 said mercury(II) compound corresponds to the formula:



wherein:

40  $\text{X}_2$  stands for alkylene including substituted alkylene, arylene including substituted arylene, or aralkylene including substituted aralkylene,

$\text{Y}$  stands for alkyl including substitute dalkyl, aryl including substituted aryl or a heterocyclic nucleus including a substituted heterocyclic nucleus, and  
45  $\text{M}$  stands for hydrogen, alkali metal, alkaline earth metal, ammonium, guanidine or an organic amine.

4. Photographic material according to claim 1, wherein  
50 in said mercury(II) compound is present in an amount of from 0.1 mg. to 30 mg. per mole of silver halide.

5. Photographic light-sensitive silver halide material according to claim 1, wherein said material also includes a stabilizer of the hydroxytriazolopyrimidine type.

6. Photographic light-sensitive silver halide material according to claim 1, wherein said material also includes a development accelerator of the polyoxyalkylene type.

7. Photographic light-sensitive silver halide material according to claim 1, wherein said emulsion is a gelatino silver halide emulsion.

## References Cited

## UNITED STATES PATENTS

|           |         |                |        |
|-----------|---------|----------------|--------|
| 2,728,663 | 12/1955 | Allen et al.   | 96—109 |
| 2,728,665 | 12/1955 | Leubner et al. | 96—109 |
| 2,728,666 | 12/1955 | Carroll et al. | 96—109 |
| 2,728,667 | 12/1955 | Knott et al.   | 96—109 |
| 2,732,302 | 1/1956  | Knott et al.   | 96—109 |
| 3,432,304 | 3/1969  | Saleck et al.  | 96—109 |

## FOREIGN PATENTS

|         |        |        |        |
|---------|--------|--------|--------|
| 537,023 | 2/1957 | Canada | 96—109 |
|---------|--------|--------|--------|

WILLIAM D. MARTIN, Primary Examiner

75 R. M. SPEER, Assistant Examiner